

## UNITED STATES PATENT OFFICE.

ARTHUR E. BELLIS, OF SPRINGFIELD, MASSACHUSETTS, AND CHARLES S. COLLINS, OF NEW YORK, N. Y., ASSIGNEES, BY MESNE ASSIGNMENTS, TO THE BELLIS HEAT TREATING COMPANY, OF NEW HAVEN, CONNECTICUT, A CORPORATION OF CONNECTICUT.

## POT OR CRUCIBLE.

No Drawing.

Application filed November 16, 1920. Serial No. 424,567.

To all whom it may concern:

Be it known that we, ARTHUR E. BELLIS and CHARLES S. COLLINS, citizens of United States, and residents of Springfield, county of Hampden, and State of Massachusetts, and borough of Bronx, city, county, and State of New York, respectively, have invented certain new and useful Improvements in Pots or Crucibles, of which the following is a specification.

This invention relates to pots or crucibles for use in the heat treatment of metals, and more particularly concerns such pots or crucibles as are designed for containing molten or liquid baths of metals or metal salts for the heat treatment of ferrous or non-ferrous metals at high temperatures.

In the art of heat treating metals, when treatment baths of the above character are used, it is generally customary to employ pots or containers for the bath materials which are constructed of cast metal alloys offering a high resistance to oxidization. Such alloys are usually of nickel, chromium and iron; of nickel, zirconium and iron; or of silicon, chromium and iron, as in alloys of this nature when exposed to an oxidizing atmosphere at high temperatures, a protecting oxide coating forms on the exposed surface, which acts as a protection to the metal against further oxidization and resultant deterioration or destruction.

We have determined that it is exceedingly difficult in actual practice to produce pots or crucibles of these alloys in the form of castings having a uniformly homogeneous physical structure, so that all such castings will be absolutely nonporous. With present foundry practice, it is possible by the exercise of extreme care to secure some non-porous castings. These pot castings when used at temperatures from 1200° F. to 1800° F., and containing salt baths or lead baths are known to give a useful service of from 3,000 to 6,000 hours. On the other hand, the larger percentage of such cast pots or crucibles of the same alloy material and cast under the same foundry supervision, when used for the same purpose and at the same temperatures have developed porosity during the first 300 hours of operation.

When the incipient pores of the cast metal pot or crucible are enlarged under high

temperatures to such an extent that the bath material will seep therethrough, this bath material attacks the coating of oxide on the exterior surface of the pot or crucible wall and removes the same. The protection afforded by the coating of oxide having thus been destroyed, the process of oxidization is renewed and as fast as the oxide reforms, it is dissipated and consumed by the bath material seeping through the pores of the pot wall. A continuation of this process finally results in a complete breakdown of the pot wall and the leakage of the bath material to such an extent that a new pot or crucible casting must be provided.

Among other alloy metals which have been commonly used in the art for making such cast pots, are chrome iron and chrome nickel. The former is produced under the trade name "Duraloy" and may be obtained in varying degrees of hardness and is capable of being readily machined or worked. Chrome nickel is known in the art as nichrome and likewise may be easily machined or worked in shape. It has been common practice to form pots or crucibles either in whole or in part of these alloy metals by the casting process. It will be understood that our present improvement in the art does not necessarily involve any specific composition of these alloy metals.

Crucibles of the special metal alloy castings above referred to are very expensive, and the high percentage of porous crucible castings of this character renders their use in the economical heat treatment of metal prohibitive. In so far as we are aware no process or method has yet been devised for eliminating the development of porosity in the use of such alloy crucible castings.

It is, therefore, the primary object and purpose of our present invention to provide a pot or crucible of chromium or zirconium metal alloy which entirely eliminates the inherent deficiencies of the cast metal alloy crucible above referred to. To this end our invention consists in the production of a pot or crucible for the heat treatment of metals at high temperatures formed from alloys of the above character, or analogous metal alloys, offering high resistance to oxidation and characterized by the formation of a protective oxide coating

on the pot wall at high temperatures. This metal alloy is forged, rolled, pressed, or otherwise wrought and from the wrought alloy the pot or crucible of the desired 5 shape and capacity is fashioned. We have found from actual experience that pots or crucibles of this character, in contradistinction to a pot of the same metal alloy in the form of a casting, is absolutely non- 10 porous and effectually prevents deterioration of the pot structure in service. While the serious objection to such cast metal alloy pots has been generally recognized in the art, in so far as we are aware, such pots 15 have never been produced from wrought, alloy metals for the purpose of overcoming the objection. Our improved wrought metal alloy pot or crucible in actual practice is capable of withstanding exceedingly high 20 temperatures and of giving continuous service for a maximum period of 6,000 hours. As all of the pots or crucibles thus produced have a uniformly homogenous structure, waste is wholly eliminated so that the 25 initial cost of producing the pots or crucibles is materially reduced, in addition to the economy realized in the actual use of the pots.

In the preceding paragraph and in the 30 claims, the word "wrought" is used in a comprehensive sense as including various ways of working metal as distinguished from merely forming it into a casting.

As an alternative embodiment of our invention, we propose to use a crucible having an external wall of the cast metal alloy, as heretofore produced, which has a high 35 resistance to oxidizing atmospheres at high temperatures. Within this external wall of 40 the crucible, an internal wall or liner is placed as in the crucible structures disclosed in the pending applications for 45 patents of Arthur E. Bellis, filed December 10, 1919, Serial No. 343,760, or Charles S. 50 Collins, filed August 30, 1920, Serial No. 406,870. The internal wall or liner of the crucible may be constructed of pressed steel 55 or pressed or wrought iron, both of which can be produced with practical certainty of the absence of incipient pores. Therefore, as 60 the bath material cannot pass through the internal wall or liner, there will be no deterioration of the expensive alloy metal of which the external wall is formed, even 65 though the latter may develop porosity. After the oxide coating forms upon the outer surface of the external wall it will be protected against further oxidation.

Again, we may use a pot or crucible having 70 an internal wall or liner of cast iron or cast steel and while the possibility exists that these cast internal walls may develop porosity when subjected to high temperatures, they may be readily removed 75 and replaced by a new liner. The cost of

such replacement is considerably less than would be incurred in the replacing of the more expensive cast crucible of the special oxidization resisting alloys. With careful foundry supervision sufficient non-porous 70 cast iron or cast steel liners may be obtained to warrant the use of this construction.

Further, we have found it possible to use an internal liner of cast steel, cast iron or pressed steel and a cast steel or cast iron external body. Owing to the fact that deterioration by oxidization will take place entirely on the surface of the external wall, the internal wall or liner may be cast relatively thin which of course would not be permissible if this liner had to withstand deterioration from oxidization. In present foundry practice a thin wall of cast iron or steel may be more readily cast with certainty of a non-porous structure than a thick wall pot or crucible.

Of course, it is very well known in the art that a pot or crucible of cast steel or iron 90 will oxidize on its exterior surface, and such pot or crucible may be non-porous. But, the thin oxide coating which forms on the wall readily scales off and the process of oxidization goes on practically continuously until the metal structure is entirely consumed. The chromium or zirconium oxide of the alloy metals herein mentioned does not, however, scale off but adheres with great tenacity and, therefore, provides a 95 protective coat on the exterior of the pot wall which it is desirable to retain. Accordingly, it will be appreciated that we have made a very distinct advance in the art in producing such pots or crucibles from a wrought alloy metal which is absolutely 100 non-porous, instead of in the form of a casting which develops porosity after a short period of use, resulting in the seepage of the bath materials and the destruction of the protective oxide coating.

What we claim is:

1. A pot or crucible for the heat treatment of metals at high temperatures, composed of a wrought, non-porous metal alloy highly resistant to oxidizing atmospheres.
2. A pot or crucible for use in the heat treatment of metals at high temperatures composed of wrought metal having a substantially non-porous physical structure and characterized by the formation on the outer exposed surface of the pot or crucible of a tenacious oxide coating when the crucible wall is subjected to a high temperature in the presence of oxidizing atmosphere.
3. A pot or crucible for use in the heat treatment of metals at high temperatures comprising an external wrought metal alloy wall having a substantially non-porous physical structure and offering high resist-

ance to oxidizing atmospheres at high temperatures, and an inner pot wall of cast ferrous metal.

4. A pot or crucible for use in the heat treatment of metals at high temperatures composed of a wrought non-porous metal alloy having as one of its constituents a metal of the chromium group.

5. A pot or crucible for use in the heat treatment of metals at high temperatures composed of a wrought non-porous metal

alloy having as one of its constituents a metal of the chromium group and characterized by the formation of a permanent oxide coating on the exposed surface of the pot or crucible in the presence of an oxidizing atmosphere.

In testimony that we claim the foregoing as our invention, we have signed our names hereunder.

ARTHUR E. BELLIS.  
CHARLES S. COLLINS.